

2,991,182

## FLAMEPROOFING COMPOSITION

Charles M. Shaw, Albany, Calif., assignor to California Research Corporation, San Francisco, Calif., a corporation of Delaware

No Drawing. Filed Dec. 21, 1959, Ser. No. 860,686

3 Claims. (Cl. 106—15)

This invention relates to novel compositions for the flameproofing of normally flammable articles. More particularly, the invention is concerned with superior new wood flameproofing compositions containing thiophosphorus compounds and unique combinations thereof.

Wood is employed extensively in many present day structures because it is often more available and easier to work with on location than other materials. Bridges, telephone poles, railroad trestles, loading docks and marine wharves are illustrative of some of the more common uses. In such applications, it is generally desirable to treat the wood with preservative oils to prevent decay or other deterioration. Unfortunately, the treated wood structures are even more susceptible to damage by fire because of the flammable nature of the preservative oil which is cumulative to the normal combustibility of the wood.

Fire damage is also a matter of concern in many inflammable articles other than wooden structures. For example, cotton and similar fibers used in the manufacture of cloth such as canvas for tents and tarpaulins are well known for their flammability. Such articles also are commonly treated with preservatives which add to the normally flammable character of the fibers.

It has now been found that flammable articles are effectively flameproofed by impregnation with a superior new composition comprising a major proportion of liquid vehicle, more particularly a preservative oil, and at least 5% by weight of a member of the groups consisting of (1) reaction product of phosphorus pentasulfide and pinene, (2) zinc dialkyl dithiophosphate containing from 3 to 8 carbon atoms in each of the alkyl groups and zinc dialkylphenyl dithiophosphate containing from 14 to 24 carbon atoms in each of the alkylphenyl groups, and (3) combination of members of each of group (1) and group (2), said combination consisting of from 10 to 90% by weight of reaction product and from 10 to 90% by weight of zinc dithiophosphate.

The normally inflammable nature of wood or other such flammable articles is remarkably inhibited by treatment with the flameproofing compositions of this invention. The unique combination of thiophosphorus compounds in the compositions provides a much greater fire retarding effect than would be expected from the performance of either one of the thiophosphorus compounds alone.

The term "flameproof" is used in this description in its commonly accepted sense and refers to the treatment of the article so that it is resistant to the propagation of flame once the ignition source has been removed. This use is consistent with the definition of the term in the ASTM standards yearbook for 1944 under Test D626-41T.

The liquid vehicles and preservative oils of the compositions according to this invention are primarily for the purpose of providing a suitable carrier for applying the thiophosphorus composition to the article being treated. Aqueous compositions are useful. Preferably, however, the liquid vehicle is an oil. The oil may be designed to evaporate and leave the flameproof composition of the phosphorus compounds as a residue in the treated article, as in the case of a light "thinner" or petroleum naphtha. It may be designed to penetrate and serve as a preservative or it may remain largely on the surface and serve

as a finish or protective coat. For example, linseed or other vegetable oils and natural or synthetic resins may be used to form flameproof coatings. Various petroleum and coal tar derived oils, such as cresols, aromatic petroleum extracts, medium boiling fuels of the diesel oil and furnace oil type, and heavier fuels, for example, topped naphthenic crude oil may be used to penetrate and preserve the article treated. The wood preservative oils having pesticidal and fungicidal properties such as creosote and petroleum hydrocarbons containing pentachlorophenol, and combinations thereof, are presently preferred.

The reaction product of phosphorus sulfide and pinene is the material resulting from the condensation of a terpene such as present in turpentine with a phosphorus pentasulfide. In the preparation of these condensation products, the ratio of turpentine to phosphorus pentasulfide is usually within the range of about 1:1 to about 3:1. The condensation is exothermic and proceeds spontaneously after heating slightly to initiate the reaction. Usually, the turpentine or other pinene or terpene containing material is heated to about 200° F. and the phosphorus pentasulfide is added slowly with stirring. Cooling may be employed if necessary to avoid undesirably high temperatures in excess of 300° F. In the process, addition agents such as aliphatic alcohols, for example, lauryl alcohol may be combined with the turpentine and phosphorus pentasulfide.

Illustrative thiophosphate compounds for present purposes include the metal salts of thiophosphates prepared by the reaction of phosphorus pentasulfide with an aliphatic alcohol or an alkyl phenol. Such reactions are straightforward and excess unreacted materials are readily removed by conventional separation methods, for example, filtration, distillation and the like. The alcohols and phenols, or mixtures thereof, are usually reacted with phosphorus pentasulfide at temperatures of from about 200 to 300° F. The suitable aliphatic alcohols contain from 1 to 16 carbon atoms and preferably 3 to 8 carbon atoms. The alkyl phenols contain from 8 to 24 carbon atoms and preferably 14 to 24 carbon atoms. The dialkyl dithiophosphates formed from the aliphatic alcohols are preferred over the alkylphenyl analogs from the standpoint of effectiveness and economy of raw materials. The metal salt of the phosphorus sulfide reaction product is conveniently formed by the addition of the corresponding metal oxide to the reaction product. The zinc salts are preferred. No special conditions are required, although heating and stirring are usually employed to effect complete reaction.

The pinene-phosphorus sulfide reaction products and the metal dithiophosphates of the flameproofing compositions, as mentioned above, are generally known as lubricating oil additives. They are described in considerable detail in various texts on lubricating oil additives. A brief description of such additives is to be found at pages 167 to 178 of "Motor Oils and Engine Lubrication" by Georgi, published in 1950 by Reinhold Publishing Corporation, New York, New York. So far as is known, such compounds have not been suggested in the form of the present compositions and concentrates, nor have they been proposed for use with preservative oils as flameproofing compositions.

The combination of phosphorus pentasulfide and pinene reaction product and the zinc dithiophosphate, as mentioned above, is surprisingly effective. It may vary in proportions so long as there is at least 10% by weight of each of the compounds in the combination. For present purposes, the combination of thiophosphorus compounds satisfactorily ranges from 10% to 90% by weight of the combination as phosphorus pentasulfide-pinene reaction product and 10 to 90% by weight as zinc dithiophosphate.

Ordinarily, maximum benefit of the combination of additives is obtained with 40 to 60% by weight of each in the combination.

The phosphorus pentasulfide-pinene reaction product and zinc dithiophosphate and their combination in the wood preservative oil are used in minor amounts sufficient to inhibit or retard burning of the treated wood. At least 5% by weight of the compounds on the basis of total composition is ordinarily desirable, particularly in the treatment of wood. Usually not more than 20 or 30% of the thiophosphate compounds is required for effective flameproofing.

In accordance with the present invention, concentrates of the combination of thiophosphorus compounds are also provided as particularly suited for the preparation of the flameproofing compositions from wood preservative oils that may be available at the particular time and place of treatment. These concentrates contain at least 60% by weight of the combination of phosphorus pentasulfide-pinene reaction product and zinc dithiophosphates. Ordinarily, not more than 90% of the combination is used. The balance of the concentrate is usually chosen from any of the typical petroleum hydrocarbon oils such as diesel fuel, creosote, etc. For present purposes, a liquid aromatic petroleum hydrocarbon fraction obtained by sulfur dioxide extraction is found particularly satisfactory. The preferred concentrates contain from 40 to 60% by weight of each of the two different thiophosphorus compounds, the total, of course, not exceeding the 90% by weight already mentioned.

The following compositions are illustrative of the invention:

prepared is found to give excellent fire retarding properties to wood in the standard tests, as described below.

The standard crib burning tests show the effect of the flameproofing compositions on a field scale. In the crib tests, the treated timber being evaluated is arranged in the form of a square crib. The timber is cut from thoroughly air-seasoned 7 in. x 9 in. x 8 ft. Douglas fir cross ties having a moisture content of 11 to 13%. The ties are cut into pieces of three sizes: 4 1/4 in. x 7 in. x 8 ft. rough, 4 in. x 4 in. x 24 in. smooth on four sides and 2 in. x 4 in. x 2 in. smooth on four sides. The number of pieces of each size treated with the flameproofer is approximately double the number used. The pieces with the highest and the lowest retentions are rejected. The 4 1/4 in. x 7 in. pieces are treated in the original 8 ft. length. Before testing, 8 inches are cut off the ends of each piece and the remainder is cut in half. Thus, the pieces actually burned are 4 1/2 x 7 in. by 40 in. The 2 x 4 and 4 x 4 pieces are treated and burned in the 24 in. length.

In these tests, a comparison is made by the use of four different treatments. The treatments are: (1) straight creosote, (2) an aqueous solution containing about 8% of water soluble salts consisting of 10% diammonium phosphate, 60% ammonium sulfate, 20% sodium tetraborate anhydrous and 10% boric acid, (3) a commercially available flameproofing composition consisting of 88% creosote and 12% tricresylarylphtosphate (8.6% phosphorus), and (4) a composition according to the present invention consisting of 10% by weight of the concentrate of Example I, and 90% by weight creosote.

The cribs are set up as hollow squares approximately 4 ft. high. The cribs of the 4 1/4 in. x 7 in. x 40 in. pieces

TABLE I

| Composition | Carrier or Wood Preservative     | Percent | Compound (1)                              | Percent | Compound (2)                                               | Percent |
|-------------|----------------------------------|---------|-------------------------------------------|---------|------------------------------------------------------------|---------|
| 1.....      | (Diesel Fuel Oil.....            | 90.0    | Zinc ditetradecylphenyl dithiophosphate.  | 4.25    | Turpentine-P <sub>2</sub> S <sub>5</sub> Reaction Product. | 4.25    |
| 2.....      | (Pentachlorophenol.....          | 1.5     | Zinc butyl hexyl dithiophosphate.         | 1.0     | Pinene-P <sub>2</sub> S <sub>5</sub> Reaction Product.     | 9.0     |
| 3.....      | Creosote.....                    | 90.0    | Zinc dodecyl dithiophosphate.             | 10.0    | do.....                                                    | 5.0     |
| 4.....      | Grade 1 Naphthenic Fuel Oil..... | 85.0    | Zinc butyl amyl dithiophosphate.          | 2.5     | do.....                                                    | 2.5     |
| 5.....      | (Diesel Fuel.....                | 90.0    | Zinc dodecylphenyl hexyl dithiophosphate. | 18.0    | Turpentine-P <sub>2</sub> S <sub>5</sub> Reaction Product. | 2.0     |
| 6.....      | (Pentachlorophenol.....          | 5.0     | Zinc methyl ethyl dithiophosphate.        | 2.0     | Pinene-P <sub>2</sub> S <sub>5</sub> Reaction Product.     | 3.0     |
| 7.....      | Creosote.....                    | 80.0    | Zinc ditetradecylphenyl dithiophosphate.  | 5.0     | Turpentine-P <sub>2</sub> S <sub>5</sub> Reaction Product. | 5.0     |
| 8.....      | No. 2 Furnace Oil.....           | 95.0    | Zinc butyl amyl dithiophosphate.          | 10.0    | do.....                                                    | 10.0    |
| 9.....      | Water.....                       | 85.0    | Zinc ditetradecylphenyl dithiophosphate.  | do..... | Pinene-P <sub>2</sub> S <sub>5</sub> Reaction Product.     | 5.0     |
| 10.....     | Creosote.....                    | 90.0    | Zinc butyl amyl dithiophosphate.          | do..... | do.....                                                    | 10.0    |
| .....       | do.....                          | 90.0    | Zinc butyl amyl dithiophosphate.          | do..... | do.....                                                    | 5.0     |
| 10.....     | Boiled Linseed Oil.....          | 90.0    | Zinc butyl amyl dithiophosphate.          | 5.0     | do.....                                                    | 5.0     |

The effectiveness of the flameproofing compositions according to the present invention is further illustrated by the following examples. In these examples, the proportions unless otherwise specified are given on a weight basis:

#### Example 1

A flameproofing composition is prepared consisting of 90% by weight of creosote and 10% by weight of a typical concentrate of a combination of thiophosphorus compounds as described above. In this instance, the concentrate consists of 42.5% by weight of zinc butyl hexyl dithiophosphate, 42.5% by weight of phosphorus pentasulfide and  $\alpha$ -pinene reaction product and 15% by weight of a medium boiling liquid aromatic petroleum hydrocarbon  $\text{SO}_2$  extract. The flameproofing composition thus

are open on top while the cribs of the 4 x 4 and 2 x 4's are closed on top. The ignition is by means of a gasoline fire. In the testing of the 4 1/2 x 7 pieces, an aluminum pieplate with 1/2 pt. of gasoline is set in the center of each crib and the 2 cribs tested together are ignited at the same time. In the 4 x 4 cribs, the gasoline is held in 1 qt. cans for about 2 minutes, at which time the cans are tipped over to ignite the wood. Temperatures reached in the fire are measured and go as high as about 2,000° F. after about 10 minutes down to about 200° F. after 40 minutes of burning time. In the tests, the time for the fire to go out is measured, as well as the time for any collapse of the timbers. The weight of the remainders of the pieces after scraping off char is also measured.

The results of the tests are given in the following table.

TABLE II

| Treatment Composition           | Creosote Or Solution, lbs./ cu. ft. | Percent Weight Lost In Burning | Time (min.) For Fire To Go Out Or To Collapse of Crib |
|---------------------------------|-------------------------------------|--------------------------------|-------------------------------------------------------|
| Set No. 1—4½" x 7" x 40" pieces |                                     |                                |                                                       |
| (1)                             | 15.4                                | 100                            | Collapsed 104'.                                       |
| (2)                             | 15.8                                | 38                             | Out in 45'.                                           |
| (3)                             | 15.5                                | 42                             | Do.*                                                  |
| (4)                             | 14.9                                | 34                             | Out in 33'.                                           |
| Set No. 2—4" x 4" x 24" pieces  |                                     |                                |                                                       |
| (1)                             | 20.4                                | 100                            | Collapsed.                                            |
| (3)                             | 23.0                                | 27                             | Out in 34'.                                           |
| (4)                             | 22.7                                | 28                             | Out in 29'.                                           |
| Set No. 3—2" x 4" x 24" pieces  |                                     |                                |                                                       |
| (1)                             | 25.2                                | 100                            | Collapsed 35'.                                        |
| (3)                             | 25.4                                | 100                            | Collapsed 48'.                                        |
| (4)                             | 25.2                                | 100                            | Collapsed 66'.                                        |

\*Very small flames remained at end of a few places.

It is readily seen from the above test results that the thiophosphate flameproofing compositions of this invention are remarkably more effective than commercial compositions presently in use. The need for flameproofing compositions is clearly shown in the test results. Wood treated with wood preservative oil alone such as the creosote is completely consumed in the test. Employing the flameproofing compositions of this invention, it is seen that a substantial amount of the flameproofer is retained by the treated wood, there is less weight lost in the wood and the flames burn themselves out and the fire is self-extinguished in a shorter period of time. Thus in each of the three critical evaluations of the effectiveness of typical flameproofing agents, the compositions of the invention are found to be superior.

#### Example II

In this example, the widely accepted panel fire test is employed to evaluate flameproofing compositions according to this invention. In the tests, analogous flameproofing compositions employing the two different thiophosphorus compounds separately and in combination are carried out to show the effectiveness of the compositions. The improvement obtained when the thiophosphorus compounds are employed in combination in accordance with a preferred embodiment of the present invention is also shown.

Douglas fir panels are made up of three pieces of 2 in. x 10 in. x 14 ft. long wood and two pieces of 2 in. x 6 in. x 14 ft. long. The panels are treated under the usual temperature and pressure conditions with 10% by weight of each flameproofing agent in a 50:50 mixture of creosote and residual fuel oil (topped naphthenic crude). The panels are allowed to weather for a period of at least 60 days. Following this, the panels are installed as part of the flooring in a mock-up railroad trestle section. The burning of the panels is accomplished by the ignition of tumbleweed stacked tightly under the trestle section. During the burning, temperatures between about 1500° F. and 1600° F. are reached.

The following table shows the results of the tests. In Composition No. 1, the flameproofing agent added to the 50:50 creosote and residual fuel is 85% by weight alpha-pinene and phosphorus pentasulfide reaction product in combination with 15% by weight of medium boiling petroleum aromatic hydrocarbon extract. The agent of Composition No. 2 is 85% by weight zinc butyl hexyl dithio-

phosphate and 15% extract. Composition No. 3, illustrative of the preferred flameproofing compositions of the present invention, uses a typical concentrate consisting of 42.5% by weight alpha-pinene and phosphorus pentasulfide reaction product, 42.5% by weight zinc butyl hexyl dithiophosphate and 15% by weight aromatic hydrocarbon extract.

TABLE III

|    |                               | No. 1 | No. 2 | No. 3 |
|----|-------------------------------|-------|-------|-------|
| 10 | Retention, Pounds per cu. ft. | 20.69 | 20.31 | 22.30 |
| 15 | Wood Burning, Minutes         | 20    | 12    | 11    |
|    | Weight Before Burning, lb.    | 450½  | 436½  | 442½  |
|    | Weight After Burning, lb.     | 435   | 425   | 434   |
|    | Weight Lost, Pounds           | 15½   | 11½   | 8½    |
|    | Wind, m.p.h.                  | 3     | 3     | 3     |
|    | Depth of Char, inches         | ½     | ½     | ½     |
|    | No. of Panels Treated         | 2     | 2     | 2     |

The above test results show conclusively that remarkable flameproof properties are obtained by treatment with the compositions according to the invention.

It will also be seen from the test results that Composition No. 3 in particular containing the combination of thiophosphorus compounds in accordance with the preferred embodiment of the invention is surprisingly superior to Compositions 1 and 2 containing the single thiophosphorus compounds. Considerably more of Composition 3 is retained in the wood compared to Compositions 1 and 2. The burning time is definitely shorter and the weight loss of the wood due to burning is approximately 30% less than the best of the other two compositions, namely Composition No. 2.

I claim:

1. A composition for flameproofing consisting essentially of wood preservative oil and from about 5 to 30% by weight of the combination of (1) reaction product of phosphorus pentasulfide and pinene and (2) zinc dithiophosphate selected from the group consisting of zinc dialkyl dithiophosphate containing from 3 to 8 carbon atoms in each of the alkyl groups and zinc dialkylphenyl dithiophosphate containing from 14 to 24 carbon atoms in each of the alkylphenyl groups, said combination consisting of from 10 to 90% by weight of reaction product and from 10 to 90% by weight of zinc dithiophosphate.
- 45 2. A composition for flameproofing consisting essentially of wood preservative oil and from about 5 to 30% by weight of the combination of (1) reaction product of phosphorus pentasulfide and alpha-pinene and (2) zinc butyl hexyl dithiophosphate, said combination consisting of from 10 to 90% by weight of reaction product and from 10 to 90% by weight of zinc dithiophosphate.
- 50 3. A concentrate useful in the preparation of wood flameproofing compositions, said concentrate consisting essentially of a liquid petroleum hydrocarbon aromatic extract and from about 60 to 90% by weight of the combination of (1) reaction product of phosphorus pentasulfide and pinene and (2) zinc dithiophosphate selected from the group consisting of zinc dialkyl dithiophosphate containing from 3 to 8 carbon atoms in each of the alkyl groups and zinc dialkylphenyl dithiophosphate containing from 14 to 24 carbon atoms in each of the alkylphenyl groups, said combination consisting of from 10 to 90% by weight of reaction product and from 10 to 90% by weight of zinc dithiophosphate.
- 55 4. A composition for flameproofing consisting essentially of wood preservative oil and from about 5 to 30% by weight of the combination of (1) reaction product of phosphorus pentasulfide and pinene and (2) zinc dithiophosphate selected from the group consisting of zinc dialkyl dithiophosphate containing from 3 to 8 carbon atoms in each of the alkyl groups and zinc dialkylphenyl dithiophosphate containing from 14 to 24 carbon atoms in each of the alkylphenyl groups, said combination consisting of from 10 to 90% by weight of reaction product and from 10 to 90% by weight of zinc dithiophosphate.
- 60 5. A composition for flameproofing consisting essentially of wood preservative oil and from about 5 to 30% by weight of the combination of (1) reaction product of phosphorus pentasulfide and pinene and (2) zinc dithiophosphate selected from the group consisting of zinc dialkyl dithiophosphate containing from 3 to 8 carbon atoms in each of the alkyl groups and zinc dialkylphenyl dithiophosphate containing from 14 to 24 carbon atoms in each of the alkylphenyl groups, said combination consisting of from 10 to 90% by weight of reaction product and from 10 to 90% by weight of zinc dithiophosphate.

65

#### References Cited in the file of this patent

#### UNITED STATES PATENTS

- 2,344,393 Cook et al. Mar. 14, 1944  
 2,358,305 Cook et al. Sept. 19, 1944  
 70 2,368,000 Cook et al. Jan. 23, 1945